

1

3,067,272

CATALYTIC DEHYDROGENATION PROCESS  
Hervey H. Voge, Berkeley, Calif., assignor to Shell Oil Company, New York, N.Y., a corporation of Delaware  
No Drawing. Filed Dec. 30, 1960, Ser. No. 79,527  
11 Claims. (Cl. 260—680)

This invention relates to a new catalytic dehydrogenation process which is particularly useful for the production of butadiene and/or isoprene.

The most used commercial process for the production of butadiene and isoprene involves the catalytic dehydrogenation of butylene and amylanes with an iron oxide catalyst promoted with sizeable amounts of potassium carbonate and generally a small amount of chromium oxide. This process requires that the dehydrogenation be effected in the presence of a large excess of steam. Although the patent literature indicates steam to olefin mole ratios as low as 1 to 1, it is well known that much higher ratios are required for efficient operation. In commercial practice this ratio is above at least 8 to 1 and generally around 12 to 1.

In the hitherto used commercial process quite high reaction temperatures are required. The range used commercially generally falls between about 590 and 650° C. At these high temperatures and in the presence of the large amounts of steam the activity of the catalyst is maintained by the continuous removal of carbonaceous deposits from the catalyst by the steam-carbon reaction which is catalyzed by the potassium carbonate in the catalyst. Thus the potassium carbonate is an essential ingredient.

An important factor in the production of butadiene and/or isoprene by dehydrogenation is the selectivity of the dehydrogenation process. The percent selectivity is defined as 100 times the moles of desired product produced divided by the moles of feed stock destroyed or otherwise converted. In order to obtain a reasonable selectivity the prior commercial process requires the use of low pressures. Generally pressures between about 5 and 25 p.s.i.a. are used. This necessitates large equipment and complicates the recovery of the product. At these low pressures and under otherwise near optimum conditions, a selectivity around 80% may be obtained at a total conversion around 20% in the dehydrogenation of butylene to butadiene. The operations are sometimes conducted under conditions of temperature and space velocity to obtain conversions as high as about 35%, but generally somewhat lower conversions are preferred because the selectivity drops sharply as the conversion is increased. At 40% conversion the selectivity may be only 50-60%. Thus, one of the major shortcomings of the hitherto used process is that the conversion must be limited to quite low values (about 25%) and this requires the working up of large amounts of material to recover the product and requires a sizeable recycle which further increases the size of the equipment.

One of the reasons for the inability of the presently used commercial process to operate at higher conversion is that the reaction, which (for the production of butadiene from butene-1) may be illustrated as follows:



is inhibited by the hydrogen liberated. If the hydrogen were removed much higher conversions could be used.

One further shortcoming of the present commercial process is that due to the content of potassium carbonate in the catalyst, the catalyst is very hygroscopic and becomes soft if exposed to the atmosphere. This introduces difficulties in loading the reactors and also other inconveniences.

2

The object of the present invention is to provide a new and improved process for the catalytic dehydrogenation of aliphatic olefins, both acyclic and alicyclic, which contain at least four non-quaternary contiguous carbon atoms, such as normal butylene, tertiary amylanes, cyclopentene, and similar higher olefins having up to 6 or 7 carbon atoms, to corresponding polyolefins, including diolefins, which process has one or more of the following advantages:

- 10 (1) The process may be operated with comparatively little or no steam while still retaining the activity of the catalyst at a high level.
- (2) The process may be operated at considerably lower temperatures. Whereas it is important to quickly quench 15 the reaction product from the quite high reaction temperature to a safe temperature in the hitherto used commercial process, this is not essential in the process of the present invention where lower temperatures can be used.
- (3) Potassium carbonate is not an essential ingredient 20 in the catalyst and in fact its presence is not recommended. Consequently the difficulties due to hygroscopicity of the catalyst are avoided.
- (4) The process may be effected at comparatively higher pressures, thereby allowing smaller equipment to 25 be used and facilitating the recovery of the product.
- (5) The process may be operated at higher conversions without sacrifice of the selectivity. This last is considered the most important of the advantages mentioned.
- 30 In general outline these objects are obtained by the process of this invention, in which process a vaporized feed stream containing the olefin reactant to be dehydrogenated is contacted together with certain specified amounts of oxygen and preferably a small amount of 35 steam at comparatively low temperatures between about 300° C. and 600° C. with a catalytic material containing indium compound in catalytically active amounts and the resultant vaporous product is treated in appropriate ways to recover the desired dehydrogenation product.

40

## FEED STOCK

The process of the present invention is principally of value at present for the dehydrogenation of normal butylenes to butadiene and/or tertiary amylanes to isoprene 45 but it can also be used to dehydrogenate cyclopentene to cyclopentadiene, normal amylanes to piperylene and higher olefins, e.g., hexenes and heptenes, to the corresponding more unsaturated products. The normal butylene may be butene-1 or butene-2, either cis or trans, or a mixture of normal butylenes such, for example, as 50 can be separated from the products obtained in the cracking of petroleum oils or by the catalytic dehydrogenation of normal butane. The tertiary amylene may be any one or a mixture of the amylanes having one 55 tertiary carbon atom. The feed stock may contain inert diluents such as any paraffinic or naphthenic hydrocarbon having up to about 10 carbon atoms.

One of the principal features of advantage of the present invention is that considerable amounts of propylene and isobutylene may be present in the feedstock, thereby eliminating the requirement for separating the feed stream to remove these hydrocarbons therefrom. It will be appreciated that although the catalytic material of the present invention does not produce any substantial 60 amount of oxygenated organic materials under the conditions specified herein, it is nevertheless advantageous to maintain materials which may act only as inert diluents at a reasonable minimum for economic reasons.

70

## STEAM

The feed stock is preferably catalytically dehydrogenated in the presence of added steam, but it is to be em-

phasized that the presence of added steam is only a small benefit and is not essential. Recommended proportions of steam are from about 0.1 to 2 moles per mole of reactant, but as indicated, larger amounts can be used if desired and, on the other hand, steam can be altogether omitted.

### OXYGEN

In the process of the present invention a certain amount of oxygen is passed with the feed stock through the reaction zone. Recommended amounts are from about 0.3 to 2.0 moles per mole of olefin reactant. The stoichiometric quantity is 0.5 mole per mole of olefin. It is preferred to use a stoichiometric excess, e.g., around 1 mole per mole of olefin. The oxygen may be supplied as pure or substantially pure oxygen, or air.

It is generally preferred to maintain the concentration of oxygen in the reactant mixture entering the reactor below about 12 v. percent although somewhat higher concentrations may be used if the concentration of the olefin reactant is at least about 10 v. percent when operating at 30 p.s.i.g., at least 15 v. percent when operating at 100 p.s.i.g. and at least about 20 v. percent when operating at 300 p.s.i.g. Thus when using pure oxygen it is frequently desirable to dilute the mixture with an inert or substantially inert diluent which may be steam, vapors or paraffin hydrocarbons,  $\text{CO}_2$ , or the like. On the other hand, if the amount of oxygen is such that it would constitute more than about 12 v. percent of the reaction mixture the oxygen may be introduced in increments, e.g., by injecting part of the oxygen separately into the reaction zone.

### TEMPERATURE

With the preferred catalyst the dehydrogenation becomes substantial at a minimum temperature around 300° C. The preferred temperatures are between about 350° C. and 500° C. Higher temperatures up to about 600° C. can be used, but only if efficient means are provided to remove the exothermic heat of reaction. The temperatures mentioned are those near the reactor inlet. If a fixed bed of catalyst is used the temperature down stream will be several degrees, e.g., 80° C., higher.

### PRESSURE

The preferred pressure is near atmospheric, e.g. 5 to 75 p.s.i.a. On the other hand, higher pressures up to about 150 p.s.i.a. can be used and have the advantage of simplifying the product recovery.

### SPACE VELOCITY

In general the process of the present invention allows a higher space velocity to be used. Thus, comparatively small reactors and catalyst inventories can be used. For example, gaseous hourly space velocities up to about 20,000 may be employed while still obtaining reasonable conversions. Gaseous hourly space velocity, abbreviated GHSV, is defined as the volume of total feed vapor calculated under standard condition (STP) passed per hour per unit volume of the catalyst bed. A wide range of space velocities may be used. Generally space velocities between about 500 and 5000 are very satisfactory. Temperature, pressure, and space velocity should be jointly adjusted to obtain a conversion in the most favorable range, normally 40-90%.

### METHOD OF CONTACT

The contact of the feed vapors, oxygen and steam, if any, is preferably effected by providing the catalyst in the form of a fixed foraminous bed of particles maintained at the reaction temperature and passing the feed vapors through the bed in a continuous or substantially continuous manner. In this method of operation the partial pressure of oxygen is high (maximum) at the inlet of the catalyst bed and declines toward the outlet. The concentration of diolefin product, on the other hand, is substantially zero at the inlet of the bed and maximum at the

5

outlet. Thus, the concentration of oxygen is highest where the concentration of the desired product is lowest and the concentration of oxygen is lowest where the concentration of the desired product is highest.

It is also possible to use the catalyst in powder form, but certain precautions should be taken. Thus, the powdered catalyst (e.g., passing a 100 mesh U. S. standard sieve) can be dispersed in the reactant vapor mixture and the dispersion passed through the reaction zone. Alternatively, the reactant vapor mixture may be passed up through a fluidized bed of the catalyst. In such case the oxygen may be separately introduced into the bed.

The gaseous mixture issuing from the reaction zone may be quenched but this is normally not essential. Except in some cases when operating at the upper limit of the recommended temperatures there is little tendency for side reactions to take place. The effluent is preferably cooled by indirect heat exchange with the feed and then washed with dilute caustic to neutralize the traces of organic acid present and condense and remove the steam. If air is used to supply the oxygen the remaining mixture is preferably compressed and scrubbed with oil to separate the hydrocarbons from the nitrogen, carbon dioxide, and carbon monoxide. The hydrocarbon may be stripped from the oil and subjected to an extractive distillation or a copper ammonium acetate treatment in the known manner to separate and recover the diolefin.

### CATALYST

30 The catalyst used in the process of the present invention differs materially from those used in the commercial process mentioned above. While the catalyst used in the present process may contain some iron oxide this oxide is by no means essential and when present it is used in 35 much smaller concentrations than in the hitherto used catalysts. Also the catalyst used in the process of the present invention preferably contains no potassium carbonate, or the equivalent thereof, and the process does not depend at all upon the steam-carbon reaction to maintain catalyst activity. Nevertheless continuous operation is not only possible but also recommended.

The process of the present invention utilizes essentially a material represented herein as a composition of matter consisting of indium, oxygen and an element selected from 45 the group consisting of phosphorus, molybdenum and tungsten in combined form. A preferred composition of matter having catalytic effect in the oxidative dehydrogenation reaction described herein will be referred to hereinafter as indium phosphate ( $\text{InPO}_4$ ). A description of 50 indium phosphate is found in the Journal of the Chemical Society, 1960, pages 2452 through 2457, by Brownlow, Salmon and Wall. Whereas the designation indium phosphate ( $\text{InPO}_4$ ) is used to indicate one of the preferred 55 catalytically active materials in the present invention, the composition may vary considerably from that represented by this exact formula. The catalyst may be considered as the compound  $\text{InPO}_4$  but may, on the other hand, include substantial amounts of indium oxide ( $\text{In}_2\text{O}_3$ ) in addition thereto. At any rate, the catalytic activity of 60 the material of the invention must of necessity include a substantial amount of indium, oxygen and phosphorus, molybdenum or tungsten conveniently considered as an oxygen-containing radical and, as in the case of indium phosphate, for example, the phosphate ( $\text{PO}_4$ ) radicals 65 are visualized as being integral for the most part as  $\text{InPO}_4$  molecules. Moreover, other phosphates such as, for example, calcium phosphate, barium phosphate, or the like, may be present without deleterious effect; such materials probably function principally as inert supporting media.

70 Various means for the preparation of the catalytic materials of the present invention will suggest themselves to those skilled in the art of catalyst preparation. The following are offered for the purpose of exposition only and various modifications thereof are contemplated with-

out departure from the spirit or scope of the invention. One method for the preparation of indium phosphate, for example, involves the reaction of indium nitrate in solution with phosphoric acid and ammonium hydroxide. Another preparation involves the reaction of indium oxide with phosphoric acid. A third method comprises reacting phosphoric acid with solid indium nitrate. A fourth suggested method involves the reaction of indium nitrate in solution with a soluble phosphate followed by an appropriate manipulation of pH as required. The Brownlow et al. reference (supra) suggests a still further means for preparation of the catalytic material.

Indium molybdate and indium tungstate catalysts may be prepared from reaction of indium salts with ammonium molybdate or ammonium tungstate or the corresponding oxides. The reactions may be carried out in solution at appropriate pH or in the solid state. Indium oxide may also be employed for solid state reactions. Various other ways of preparing these catalysts will suggest themselves to those skilled in the art. It is preferred to use indium nitrate and ammonium molybdate or tungstate, as in the subsequent examples, to avoid the presence of non-volatile elements other than indium, molybdenum or tungsten. Ammonium hydroxide is a preferred alkali for precipitation, but other alkalies may sometimes be used to advantage.

Indium oxide may be prepared by oxidation of the metal, by precipitation from solutions of salts, by decomposition of nitrates or other decomposable salts, or even in certain other ways.

It is to be understood that the invention also contemplates the use of mixtures or combinations of these indium compounds, such as, for example, indium phosphomolybdate and indium phosphotungstate.

The manner of working of the catalyst is not known and no explanation of its very pronounced activity can be offered at this time. Its specificity for oxidative dehydrogenation of hydrocarbons, particularly olefins to diolefins, is especially advantageous.

The catalyst may be used with or without a filler or carrier material and may be pelleted or formed in other conventional manner. If a carrier is used it is preferably one having a good thermal conductivity and pores of relatively large size such, for instance, as pellets of alundum, crushed fire brick, pumice, or the like. A filler or binding agent in an amount up to about 50% by weight of the total may be included. Suitable materials are, for example, silica, powdered aluminum, and other inert materials.

#### Example I

An indium phosphate catalyst was prepared as follows. Indium metal was dissolved in 3 molar nitric acid, and to the solution an amount of phosphoric acid stoichiometrically equivalent to the indium was added. Ammonium hydroxide, 3 molar, was then added until the pH was 7.0. The resulting hydrogel was aged overnight, filtered off, and dried. The dry material was calcined 2 hours at 500° C. and broken to 10-20 mesh white granules. Analysis showed 12.2% P compared to 14.7% by theory for  $\text{InPO}_4$ .

#### Example II

The catalyst described in Example I was used to convert 1-butene to 1,3-butadiene in a small fixed-bed reactor at atmospheric pressure. A mixture of "air" and 1-butene with an "air"/butene ratio of 8.3 was fed to the reactor. The "air" was actually a mixture of 79.5% argon and 20.5% oxygen, since nitrogen would have interfered with the mass spectrometric analysis of the reaction product stream. The results are shown in the following tabulation. Here the GHSV is the total gaseous hourly space velocity in volumes of gas (0° C., 760 mm.) per volume of catalyst per hour. The selectivity to butadiene is the percentage of the converted 1-butene that was transformed to butadiene. The balance of the converted

1-butene went chiefly to  $\text{CO}_2$  and CO, with selectivities to oxygenated compounds such as methyl vinyl ketone in the order of 1% or less.

| 5   | Maximum Temperature, ° C. | GHSV  | Conversion, percent |                              | Selectivity to $\text{C}_4\text{H}_6$ , percent |
|-----|---------------------------|-------|---------------------|------------------------------|-------------------------------------------------|
|     |                           |       | of $\text{O}_2$     | of 1- $\text{C}_4\text{H}_6$ |                                                 |
| 400 |                           | 3,360 | 35                  | 21                           | 60                                              |
| 430 |                           | 3,360 | 65                  | 44                           | 67                                              |
| 440 |                           | 6,720 | 42                  | 36                           | 72                                              |
| 465 |                           | 3,360 | 88                  | 63                           | 61                                              |
| 490 |                           | 3,360 | 98                  | 72                           | 61                                              |

#### Example III

15 The same catalyst described in Example I was used to convert 2-methyl-2-butene to isoprene. A helium-oxygen mixture was fed in lieu of air. Results were as follows:

| 20  | Maximum Temperature, ° C. | GHSV  | $\text{He}/\text{O}_2$ | Conversion, percent |                              | Selectivity to Isoprene, percent |
|-----|---------------------------|-------|------------------------|---------------------|------------------------------|----------------------------------|
|     |                           |       |                        | of $\text{O}_2$     | of $\text{C}_5\text{H}_{10}$ |                                  |
| 333 |                           | 2,600 | 6                      | 1.6                 | 85                           | 41                               |
| 420 |                           | 3,900 | 6                      | 1.7                 | 99                           | 45                               |
| 25  | 460                       | 3,900 | 6                      | 1.7                 | 100                          | 48                               |
| 490 |                           | 3,900 | 6                      | 1.7                 | 100                          | 48                               |
| 460 |                           | 4,400 | 10                     | 2.8                 | 100                          | 35                               |
| 510 |                           | 4,700 | 3.3                    | 1.0                 | 100                          | 61                               |

30 It is to be understood that the tabulated data included herein is illustrative of results obtained at approximately atmospheric pressure.

#### Example IV

An indium phosphate catalyst was prepared by mixing 35 100 ml. of 0.413 molar  $\text{In}(\text{NO}_3)_3$  in dilute nitric acid solution with 139 ml. of 3 molar phosphoric acid, heating to 70° C., and adding 3 molar ammonium hydroxide at that temperature until a pH of 8.9 was reached. The precipitate was filtered off, washed with dilute ammonia, dried, broken to 10-20 mesh white granules, and calcined 2 hours at 500° C. This was more nearly a stoichiometric  $\text{InPO}_4$  than the catalyst of Example I.

#### Example V

45 The catalyst of Example IV was used to convert 1-butene to 1,3-butadiene as in Example II, except that the "air"/butene ratio was 5. Results were:

| 50  | Maximum Temperature, ° C. | GHSV  | Conversion, percent |                              | Selectivity to $\text{C}_4\text{H}_6$ , percent |
|-----|---------------------------|-------|---------------------|------------------------------|-------------------------------------------------|
|     |                           |       | of $\text{O}_2$     | of 1- $\text{C}_4\text{H}_6$ |                                                 |
| 425 |                           | 3,600 | 21                  | 21                           | 80                                              |
| 455 |                           | 3,600 | 39                  | 31                           | 82                                              |
| 55  | 488                       | 3,600 | 60                  | 42                           | 78                                              |
| 510 |                           | 3,600 | 79                  | 49                           | 77                                              |

Thus, activity was lower than in Example II, but selectivity was higher. Almost no acetone, acetaldehyde, acrolein, crotonaldehyde, formaldehyde, or furan was formed. 60 Conversion to methylvinylketone was less than 1% in all cases.

#### Example VI

An inium oxide was prepared by precipitation from a 0.63 molar indium nitrate solution in dilute nitric acid by addition of ammonium hydroxide to pH 7. It was washed, dried and calcined at 500° C., and the yellowish granules were tested for oxidative dehydrogenation of 1-butene under the conditions of Example V. At a maximum temperature of 440° C. the conversion of oxygen was 89%, the conversion of 1-butene was 30%, and the selectivity to butadiene was 42%. The balance of the conversion was chiefly to  $\text{CO}_2$  and CO, with 6% selectivity to acetaldehyde and 2% to acetone.

7  
Example VII

An indium molybdate-silica catalyst was prepared by precipitation from a mixture of 50 ml. of a 0.63 molar indium nitrate in dilute nitric acid solution with 47 ml. of 1 molar ammonium molybdate solution and 16 grams of Ludox silica sol (ammonium form; about 30% SiO<sub>2</sub>) by addition of ammonium hydroxide to pH 6. The precipitate was filtered off, dried, and calcined as 10-20 mesh granules. Some molybdenum was lost in the filtrate and the final creamy yellow catalyst contained In/Mo in a calculated atomic ratio of 1.03. The catalyst was tested as in Example V. At a maximum temperature of 425° C. the conversion of oxygen was 63%, the conversion of 1-butene was 36%, and the selectivity to butadiene was 66%. Conversions to oxygenated compounds other than water and CO<sub>2</sub> were less than 1%.

## Example VIII

An indium tungstate-silica catalyst was prepared by mixing 50 ml. of 0.63 molar indium nitrate solution in dilute nitric acid with 472 ml. of 0.1 molar ammonium tungstate solution and 22 g of Ludox silica sol (ammonium form; about 30% w. SiO<sub>2</sub>) and adding ammonium hydroxide to pH 6. The precipitate was filtered, dried, and calcined at 500° C. The product was pale yellow. The calculated ratio of In/w. is 2/3. The catalyst was tested as in Example V. At a maximum temperature of 485° C. the conversion of oxygen was 96%, the conversion of 1-butene was 48%, and the selectivity to butadiene was 69%. Conversions to oxygenated compounds other than water and CO<sub>2</sub> were less than 0.5%.

I claim as my invention:

1. Process for the selective oxidative dehydrogenation of a C<sub>4-7</sub> monoolefinic aliphatic hydrocarbon having no quaternary carbon atoms to produce as the major reaction product a hydrocarbon having the same number of carbon atoms but at least one more ethylenic double bond, which comprises passing the aliphatic hydrocarbon in vapor phase together with from about 0.3 to 2 moles of oxygen through a reaction zone in contact with a solid catalyst therefor consisting essentially of a composition of matter consisting essentially of indium, oxygen and an element selected from the group consisting of phosphorus, molybdenum and tungsten in catalytically effective proportions at a temperature of from about 300° C. to 600° C. and at a pressure of from about 5 to 150 p.s.i.a., and recovering the second-mentioned hydrocarbon from the reaction product.

2. Process for the selective oxidative dehydrogenation of C<sub>4-7</sub> monoolefinic aliphatic hydrocarbon having no quaternary carbon atoms to produce as the major reaction product a hydrocarbon having the same number of carbon atoms but at least one more ethylenic double bond, which comprises passing the aliphatic hydrocarbon in vapor phase together with from about 0.3 to 2 moles of oxygen through a reaction zone in contact with a solid catalyst therefor consisting essentially of indium phosphate in catalytically effective proportions at a temperature of from about 300° C. to 600° C. and at a pressure of from about 5 to 150 p.s.i.a., and recovering the second-mentioned hydrocarbon from the reaction product.

3. Process for the selective oxidative dehydrogenation of a C<sub>4-7</sub> monoolefinic aliphatic hydrocarbon having no quaternary carbon atoms to produce as the major reaction product a hydrocarbon having the same number of carbon atoms but at least one more ethylenic double bond which comprises passing the first said hydrocarbon in the vapor phase together with about an equal molar amount of oxygen through a reaction zone in contact with a solid catalyst comprising as its main active constituent indium phosphate at a temperature of from about 300° C. to 600° C., a pressure of from about 5 to 150 p.s.i.a., and recovering the second-mentioned hydrocarbon from the reaction product.

4. Process for the selective oxidative catalytic dehydro-

genation of a C<sub>4-7</sub> monoolefinic aliphatic hydrocarbon having no quaternary carbon atoms to a corresponding diolefin which comprises passing said hydrocarbon in the vapor phase together with from about 0.3 to 2 moles of oxygen through a reaction zone in contact with the solid catalyst containing as its main active constituent indium phosphate at a temperature of from about 300° C. to 600° C., a pressure of from about 5 to 150 p.s.i.a., and recovering the second-mentioned hydrocarbon from the reaction product.

5. Process for the selective oxidative catalytic dehydrogenation of a C<sub>4-7</sub> monoolefinic aliphatic hydrocarbon having no quaternary carbon atoms to a corresponding diolefin which comprises passing said hydrocarbon in the vapor phase together with from about 0.3 to 2 moles of oxygen through a reaction zone in contact with a fixed foraminous bed of catalyst containing as its main active constituent indium phosphate at a temperature of from about 300° C. to 600° C., a pressure of from about 5 to 150 p.s.i.a., and recovering the second-mentioned hydrocarbon from the reaction product.

15 6. Process for the selective oxidative catalytic dehydrogenation of a C<sub>4-7</sub> monoolefinic aliphatic hydrocarbon having no quaternary carbon atoms to a corresponding diolefin which comprises passing said hydrocarbon in the vapor phase together with an approximately equal molar quantity of oxygen through a reaction zone in contact with a solid catalyst containing as its main active constituent indium phosphate at a temperature of from about 300° C. to 600° C., a pressure of from about 5 to 150 p.s.i.a., and recovering the second-mentioned hydrocarbon from the reaction product.

20 7. Process for the selective oxidative catalytic dehydrogenation of a C<sub>4-7</sub> monoolefinic aliphatic hydrocarbon having no quaternary carbon atoms to a corresponding diolefin which comprises passing said hydrocarbon in the vapor phase together with air in an amount equivalent to from about 0.3 to 2 moles of oxygen through a reaction zone in contact with the solid catalyst containing as its main active constituent indium phosphate at a temperature of from about 300° C. to 600° C., a pressure of from about 5 to 150 p.s.i.a., and recovering the second-mentioned hydrocarbon from the reaction product.

25 8. Process for the selective oxidative catalytic dehydrogenation of a C<sub>4-7</sub> monoolefinic aliphatic hydrocarbon having no quaternary carbon atoms to a corresponding diolefin which comprises passing said hydrocarbon in the vapor phase together with from about 0.3 to 2 moles of oxygen through a reaction zone in contact with a solid catalyst containing as its main active constituent indium phosphate at a temperature of from about 350° C. to 500° C., a pressure of from about 5 to 150 p.s.i.a., and recovering the second-mentioned hydrocarbon from the reaction product.

30 9. Process for the selective oxidative catalytic dehydrogenation of a C<sub>4-7</sub> monoolefinic aliphatic hydrocarbon having no quaternary carbon atoms to a corresponding diolefin which comprises passing said hydrocarbon in the vapor phase together with from about 0.3 to 2 moles of oxygen through a reaction zone in contact with a solid catalyst containing as its main active constituent indium phosphate at a temperature of from about 350° C. to 500° C., and at about atmospheric pressure, and recovering the second-mentioned hydrocarbon from the reaction product.

35 10. Process in accordance with claim 1 wherein the catalyst consists essentially of indium molybdate.

40 11. Process in accordance with claim 1 wherein the catalyst consists essentially of indium tungstate.

45 70 References Cited in the file of this patent

UNITED STATES PATENTS

- 2,007,116 Walker et al. \_\_\_\_\_ July 2, 1935  
2,945,900 Alexander et al. \_\_\_\_\_ July 19, 1960  
2,991,321 Voge et al. \_\_\_\_\_ July 4, 1961